

May 25, 1937.

J. D. DE VRIES

2,081,227

VARIABLE RESISTANCE

Filed Oct. 5, 1934

*Fig. 1.*



*Fig. 2.*



Inventor:  
J. D. de Vries,

by  
C. F. Wunderoth  
Atty.

## UNITED STATES PATENT OFFICE

2,081,227

## VARIABLE RESISTANCE

Johan Dirk de Vries, Eindhoven, Netherlands,  
assignor to N. V. Philips' Gloeilampen-  
fabrieken, Eindhoven, Netherlands

Application October 5, 1934, Serial No. 747,075  
In the Netherlands November 4, 1933

## 2 Claims. (Cl. 201—55)

My invention relates to variable resistances comprising a resistance layer formed by heating a dispersion of a resin capable of being hardened and a conductive material until the resin has sufficiently hardened, and then surface-grinding the active surface of the layer.

The term "surface-grinding" is to be understood to mean a type of grinding in which not only slight surface irregularities and a slight amount of the surface of the layer are removed, but also by which at the same time, by exerting pressure during the grinding operation, a rubbing together occurs. In the course of this grinding operation temperatures of 100 to 200° C. may occur.

As a conductor in the dispersion, preferably carbon, for instance in the form of graphite, is used, but one may also use materials such as silver oxide. Very suitable is the product sold under the registered trade-mark "Aquadag", which consists essentially of colloidal graphite suspended in water.

Suitable resins capable of being hardened are for instance, shellac and artificial resins, for instance, phenolformaldehyde condensation products, capable of being hardened, the latter being preferably used.

The present invention has the advantage that a hard resistance layer can be obtained which makes it possible to use a spherically shaped contact body for making sliding contact therewith. Due to the hardness of the layer the sliding back and forth of this body during operation causes no excessive wearing of the resistance layer.

In fact, contact members having a comparatively large surface, for instance, in the form of a shoe were generally used hitherto with other resistance layers of this type for taking off current, in order that an excessive local pressure would not be exerted on the resistance layer and thus to avoid premature wearing out of said layer.

A contact that gives less rise to noises may be obtained, however, by using a contact body of a spherical type since in this case the contact point is exactly determined, the use of which is enabled by the invention.

It has already been suggested to give resistances a definite value by polishing. Furthermore it is known *per se* to manufacture resistance layers by means of dispersions wherein a conductor and resin capable of being hardened are dispersed. However, the special advantages that can be achieved with the combination of these

known operations were unknown up to the present.

The invention may be carried into effect by squirting the above-mentioned dispersion upon a solid insulating layer consisting of ceramic material. Furthermore it is possible to impregnate paper or thin cardboard with the dispersion followed by drying, heating and grinding.

Preferably fibrous layers provided with a hardened resin are used, which layers are known under the registered trade-marks "Pertinax", "Textolite", etc. As is well known these materials may be obtained by impregnating layers of fibers such as paper or tissues with a solution of an artificial resin capable of being hardened, followed by drying, heating and compressing.

This embodiment has the advantage that materials such as "Pertinax", "Textolite" and other similar materials are not only cheaper than insulating ceramic material, but can also be more readily manufactured in the form of a plate, and furthermore they already have, due to the pressing, a very smooth surface which is of great importance for the invention.

The invention allows this important embodiment since after application of the resistance layer at comparatively low temperatures, for instance, about 225° C. or less, one may proceed to baking in order that the organic insulating material be not attacked by high temperatures whereas the grinding operation permits the value of the resistance to be reduced exactly to the desired point.

For manufacturing potentiometers the dispersion may be applied in such a manner that the resistance layer has a logarithmic course.

The invention will be more clearly understood by reference to the accompanying drawing.

Fig. 1 is a longitudinal section of a potentiometer, and

Fig. 2 is a bottom view thereof.

In Fig. 1 a ring 1 consisting of Pertinax is provided with a resistance layer 2 obtained by squirting an alcoholic solution of phenolformaldehyde condensation products capable of being hardened in which Aquadag is dispersed. After drying, the resistance material thus applied is hardened during which operation the resistance layer becomes sufficiently hard to be ground. This grinding operation may be effected by using a rotatory smooth grinding surface under pressure due to which the value of the resistance is reduced. This grinding operation is discontinued after the resistance has attained the desired value. As a grinding material fine emery cloth may be used

and preferably a pressure of about 150 gms. per square centimeter is exerted. The grinding operation may be followed by heating to about 200° C. for about 5 to 8 minutes in order to enhance the hardness.

The Pertinax plate 1 is secured to a supporting plate 3 consisting of insulating material, on which plate the contacts 4 and 5 are mounted at the same time. The spherical contact member 7 is electrically connected to the contact 6 and is elastically mounted and secured to a plate 8 consisting of insulating material. The described parts, as well as the knob 10 by means of which the shaft may be turned, are mounted 10 on a shaft 9. Reference numeral 11 denotes a nut with the aid of which the plates 2 and 3 are fixed in the desired place. The spherical contact member 7 is preferably made of the

alloy known under the name "tombak", which is an alloy of copper and zinc containing a maximum of 18% zinc.

What I claim is:

1. A variable resistance comprising a resistance layer of a hardened resin and a conductive material, said layer having a burnished working surface, and a spherically-shaped contact point adapted to slide over said surface to take off the current. 5

2. A variable resistance comprising a resistance layer of a hardened resin and a conductive material, said layer having a rubbed smoothed working surface, and a spherically-shaped contact point of "tombak" adapted to slide over said 10 surface to take off the current. 15

JOHAN DIRK DE VRIES.